

## UNITED STATES PATENT OFFICE

1,947,463

MANUFACTURE AND TREATMENT OF  
CELLULOSE ESTERS

Henry Dreyfus, London, England

No Drawing. Application March 21, 1929, Serial  
No. 348,930, and in Great Britain April 18,  
1928

20 Claims. (Cl. 260--101)

This invention relates to the manufacture of cellulose esters of hydroxy aliphatic acids.

The cellulose derivatives are manufactured according to the present invention by the treatment 5 of cellulose or cellulose-containing material with anhydrides of hydroxy aliphatic acids. For convenience the cellulose derivatives thus obtained will be termed hereinafter hydroxyalkacetyl derivatives of cellulose. The hydroxy groups thereof 10 may be esterified, for instance with acetic anhydride, so as to form acidoxyalkacetyl derivatives of cellulose.

The acylation with the anhydrides of the hydroxy aliphatic acids may be carried to the mono-, 15 di-, or tri-acyl stage or to any intermediate stage, but the most valuable products are obtained if the reaction with the cellulose or cellulose-containing material is carried to the tri-acyl stage or to between the di- and tri-acyl stage.

20 The anhydrides to be used in the acylation may be derived from any convenient hydroxy aliphatic acids, for example glycollic acid, lactic acid, hydroacrylic acid etc. and may be prepared by any convenient method. For example they may be 25 prepared from the sodium, potassium, or other metallic salts of the acids or mixtures thereof by treatment with thionyl chloride.

As initial materials for acylation according to 30 the present invention cotton or any other celluloses or near conversion products thereof may be employed, or bamboo, esparto or wood pulps from which the lignin, pentosan, resin and like constituents have been substantially removed, as for example in sulphite pulp, soda pulp and sulphate 35 pulp.

The cellulosic materials may be treated, prior to the acylation, with organic acids in large or 40 small quantities, and particularly with lower fatty acids, such as formic or acetic acid, or with hydroxy-aliphatic acids, to increase their reactivity. Chemical pulps are preferably subjected to an alkaline purifying treatment, as described in my U. S. Patent No. 1,711,110, followed by the treatment with organic acids, prior to the 45 acylation. The alkaline purifying treatment may for example be performed with caustic alkali of low concentration, such as 3% or under, with heating or boiling, or with caustic alkali of high concentration, such as 5-10% or more, in the cold 50 or with only slight heating.

The pretreatment with organic acids may be carried out in any convenient manner. For example, the cellulosic materials may be pretreated with concentrated or dilute acids, particularly 55 formic or acetic acid, as described in my French Patent No. 565,654, or, where feasible, with the vapours of the acids, as described in my British Patent No. 263,938, the vapours being employed alone or mixed with air or other inert gas. After 60 the treatment with organic acids, the cellulosic

materials may be subjected to a stream of air or other inert gas or to suction or vacuum to remove the organic acids wholly or partially. Formic acid, except when employed in small quantities, should be substantially removed. If for the pre- 65 treatment an acid, such as acetic acid, is used which will serve as a solvent diluent in the subsequent acylation its removal is of course unnecessary. However, in pretreating with organic acids alone I have found that the best results are 70 obtained by employing either formic acid, such as 80-100% formic acid, or a mixture of formic acid with another acid, such as acetic acid and removing it before acylation.

Another type of pretreatment, which I have 75 found very efficacious for rendering the cellulosic material more reactive, is that described in my British Patent No. 312,098. The cellulosic material is treated with hydrochloric or other hydrohalide acid or with mixtures thereof. The acid 80 is most advantageously employed in a proportion of 5-10% (corresponding to about 15-30% of commercial acid in the case of hydrochloric acid). The aqueous acids may be distributed evenly over the cellulosic material, for instance by spraying 85 the material in a drum or mixer, the cellulosic material being allowed to stand with occasional turning to ensure uniform impregnation until a product capable of rapid acylation is obtained. This type of pretreatment is most valuable when hydrochloric or other hydrohalide acid is to be employed in the subsequent acylation as herein-after described. The metallic halide catalysts referred to below for use in conjunction with hydrochloric or other hydrohalide acid in the 90 acylation may moreover be used alone or together with the acid as pretreating agents.

The pretreatment with hydrohalide acids may furthermore be combined with a pretreatment with organic acids as described above, the two 100 treatments being conducted simultaneously or successively. Furthermore the pretreatment with organic acids may be combined with a pretreatment with other mineral acids for example sulphuric acid.

105 The actual acylation of the cellulose or cellulose-containing material with the anhydrides may be carried out in any convenient manner. For example it may be conducted in presence of a solvent or mixture of solvents for the cellulose derivative produced. Acetic acid or other lower fatty acids (with the exception of formic acid) may for example be employed. The invention is however not limited to the use of any particular solvent. The solvent or solvent mixture may be 110 present in any desired quantity such as 4 to 6 times the weight of the cellulose or cellulose-containing material, but cellulose derivatives of especially high viscosity can be obtained if the solvent or solvent mixture be present in an 115 120

amount greater than 6 times, say 8 to 20 times or more the weight of the cellulose or cellulose-containing material.

Again the acylation may be conducted in suspension in non-solvent liquid diluents. If desired solvents may be present in addition to the non-solvent diluents. As in the acylation carried out in presence of a solvent so that the cellulose derivative is produced in solution, the acetic acid 10 or equivalent solvent may be used in quantities in excess of 6 times the weight of the cellulose, for example, 8 to 20 times or more to obtain cellulose derivatives of high viscosity. In all such cases of using solvents in addition in carrying out 15 the acylation in suspension, the diluent should be present in sufficient quantity to prevent solution of the cellulose derivative produced.

Fibres, fabrics or the like made of or containing cotton or other cellulosic material may be 20 acylated by means of the processes of the present invention by carrying out the acylation in suspension in presence of liquid diluents.

The treatment with the anhydrides of the hydroxy aliphatic acids is preferably conducted in 25 presence of a suitable catalyst or condensing agent. For example, sulphuric acid or organically substituted sulphuric acids such as benzene sulphonic acid, bisulphates, e. g. sodium bisulphate, phosphoric acid, sulphuryl chloride, zinc 30 chloride or the like may be employed. Metallic halides, for example the chlorides, of iron (ferric), tin (stannic), manganese, copper, nickel or cobalt, used in conjunction with hydrochloric or other hydrohalide acids give useful results. Ferric 35 and stannic chlorides may be used without hydrohalide acid. The quantity of catalyst to be employed will vary with the catalyst selected and with the type of cellulosic material to be treated. Sulphuric acid should preferably be employed in 40 proportions under 15% calculated on the weight of the cellulose and especially in proportions of 1 to 10%, while the ferric chloride, stannic chloride, or other halides given above should preferably be employed in a proportion of 5 to 20% 45 on the weight of the cellulose, or if used in conjunction with hydrochloric or other hydrohalide acid both the halide itself and the hydrohalide acid should preferably be present in proportions of between 5 and 15% on the weight of 50 the cellulose.

In order to avoid degradation of the cellulose molecule the acylation is conducted at as low a temperature as possible. Temperatures not substantially exceeding 50° C., for example 20-30° C., 55 atmospheric temperatures, or temperatures below atmospheric, e. g. 0-10° C., are preferable. Ferric chloride or other of the halide catalysts given above do however permit of the acylation being conducted with moderate heating without 60 substantially impairing the qualities of the products obtained.

The following examples illustrate the invention but are not to be considered as limiting it in any way:—

85

#### Example 1

100 parts by weight of cotton cellulose are pretreated with formic acid, for example by treatment with 500-1000 parts of formic acid of about 70 85% strength, allowing to stand for some hours in the cold and hydro-extracting or by impregnating with about 15 parts of formic acid of 75-85% strength and allowing to stand for 8-12 hours. The material is then washed, centrifuged 75 and dried. The pretreated cellulose is then in-

troduced into a mixture of 600 parts of acetic acid, 500 parts of glycollic anhydride and 10 to 12 parts of sulphuric acid. If necessary slight heating may be applied to initiate the reaction but throughout the acylation the temperature should not be allowed to rise much above 50° C. When solution is complete, the cellulose glycolate may be separated from its solution by addition of a non-solvent, for example by addition of excess of water. It is soluble in diluted chloroform-alcohol and in aqueous acetone. 80 85

#### Example 2

100 parts by weight of cotton cellulose are pre-treated as in Example 1 and are then introduced 90 into a mixture of 500 parts of acetic acid, 400 parts of glycollic anhydride and 25 to 30 parts of sulphuryl chloride. Here again initial heating may be necessary. The temperature of the mixture is maintained at 60-70° C. until solution 95 is complete.

#### Example 3

100 parts by weight of cotton cellulose are impregnated with a mixture of 20 parts of ferric chloride and 20 parts of 35% aqueous hydrochloric acid and allowed to stand in the cold for 4-8 hours. The cellulose is then introduced into a mixture of 600 parts of acetic acid and 450 parts of glycollic anhydride. The acylation is effected 105 at 40-50° C. until solution is complete, when water may be added to destroy the remaining anhydride.

While the invention has been described above more particularly with reference to the production of cellulose derivatives of glycollic acid, it is also applicable to the production of derivatives of higher hydroxy-aliphatic acids. Furthermore mixed derivatives may be produced by employing another anhydride, e. g. anhydrides of acetic acid 110 and its homologues, in addition to the hydroxy-aliphatic anhydrides. The mixed derivatives may, for example, be produced by treating first with a hydroxy-aliphatic acid anhydride and then with 115 a fatty acid anhydride. 120

As stated above the hydroxyalkacyl derivatives or mixed alkacyl-hydroxyalkacyl derivatives of cellulose produced according to the present invention may be treated with esterifying agents, for example acetic anhydride, to produce derivatives in which the hydroxy groups have been wholly or partially converted into ester groups. Such derivatives may be termed acidyloxy-alkacyl derivatives or mixed alkacyl-acidyloxy-alkacyl derivatives of cellulose. For example the cellulose derivative of acetylglycollic acid may be obtained by treating the glycollic derivative of cellulose with acetic anhydride. If in treating a lower cellulose glycolate with acetic anhydride, as referred to above, the anhydride be employed in sufficient quantity, a mixed cellulose acetate-acetylglycolate results directly. 125 130 135

#### Example 4

100 parts of cotton cellulose pretreated as in Example 1 above are introduced into a mixture of 500 parts of acetic acid, 180 parts of glycollic anhydride and 10 parts of sulphuric acid. Heating 140 is applied and, after allowing the reaction to continue for about 5 hours at 20-30° C., 400 parts of acetic anhydride containing a further 5 parts of sulphuric acid are added. Thereafter the reaction is conducted as in the manufacture of cellulose acetate. The mixed cellulose acetate- 145 150

acetylglycollate is very similar in solubility and other properties to cellulose acetate.

I have further found that the cellulose derivatives made according to the present invention whether they be hydroxyalkacetyl or acidoxy-alkacetyl derivatives or the mixed derivatives containing in addition alkacetyl groups may be subjected to secondary treatments or reactions for the purpose of changing their solubilities. The secondary treatments or reactions may, for example, be carried out in presence of inorganic or organic acids or acid salts, the treatment being arrested when the required solubility has been reached. In carrying out the secondary treatments in the primary acylation solutions or suspensions, the acylation catalysts themselves are in most cases sufficient to effect any desired change in solubility properties.

*Example 5*

The primary acylation solution of Example 1 (i. e. the solution obtained before any separation of cellulose glycollate) is treated with 50-80 parts of water at a temperature of about 35° C. The cellulose glycollate becomes progressively soluble in organic solvents, e. g. acetone, containing more and more water. The treatment is stopped when the required solubility has been reached.

While the secondary or further treatments of the primary products may with advantage be conducted at ordinary or moderate temperatures, the reaction may, if desired, be quickened by heating up to relatively high or high temperatures, even up to 80 or 100° C. but in such cases the presence of free mineral acids is preferably avoided.

What I claim and desire to secure by Letters Patent is:—

1. Process for the production of cellulose esters containing hydroxyalkacetyl groups, comprising treating materials consisting essentially of cellulose with hydroxylaliphatic acid anhydrides.

2. Process for the production of cellulose esters containing hydroxyalkacetyl groups, comprising treating materials consisting essentially of cellulose with hydroxylaliphatic acid anhydrides in presence of acylation catalysts.

3. Process for the production of cellulose esters containing hydroxyalkacetyl groups, comprising treating materials consisting essentially of cellulose with hydroxylaliphatic acid anhydrides in presence of sulphuric acid.

4. Process for the production of cellulose esters containing glycolyl groups, comprising treating materials consisting essentially of cellulose with glycollic anhydride in presence of acylation catalysts.

5. Process for the production of cellulose esters containing glycolyl groups, comprising treating materials consisting essentially of cellulose with glycollic anhydride in presence of sulphuric acid.

6. Process for the production of cellulose esters containing glycolyl groups, comprising treating materials consisting essentially of cellulose with glycollic anhydride in presence of acylation catalysts and a liquid acylation medium.

7. Process for the production of cellulose esters containing glycolyl groups, comprising treating materials consisting essentially of cellulose with organic acids and then with glycollic anhydride in presence of acylation catalysts.

8. Process for the production of cellulose esters containing glycolyl groups, comprising treating materials consisting essentially of cellulose with organic acids and then with glycollic anhydride

in presence of acylation catalysts and a liquid acylation medium.

9. Process for the production of mixed cellulose esters containing glycolyl and acetyl groups, comprising treating materials consisting essentially of cellulose separately with glycollic anhydride and acetic anhydride, both in presence of acylation catalysts and a liquid acylation medium.

10. A cellulose ester in which part of the cellulose nuclear hydroxyl groups are esterified by alkacetyl groups and part by hydroxy-alkacetyl groups.

11. A cellulose acetate-glycollate in which part of the cellulose nuclear hydroxyl groups are esterified by acetyl groups and part by glycolyl groups.

12. Process for the manufacture of cellulose esters containing hydroxyalkacetyl groups, comprising treating materials consisting essentially of cellulose with hydroxy aliphatic acid anhydrides and subjecting the resulting primary hydroxyalkacetyl esters to the action of acidic substances for the purpose of changing their solubility characteristics.

13. Process for the manufacture of mixed cellulose esters containing hydroxyalkacetyl and alkacetyl groups, comprising treating materials consisting essentially of cellulose separately with an hydroxy aliphatic acid anhydride and a simple aliphatic acid anhydride both in the presence of acylation catalysts and a liquid acylation medium, and subjecting the resulting mixed primary cellulose esters to the action of acidic substances for the purpose of changing their solubility characteristics.

14. Process for the manufacture of cellulose esters containing hydroxyalkacetyl groups, comprising treating materials consisting essentially of cellulose with hydroxy aliphatic acid anhydrides and subjecting the resulting primary hydroxyalkacetyl esters to the action of the substances having mineral acidity for the purpose of changing their solubility characteristics.

15. Process for the manufacture of cellulose glycollates comprising treating materials consisting essentially of cellulose with glycollic anhydride and subjecting the resulting primary cellulose glycollates to the action of acidic substances for the purpose of changing their solubility characteristics.

16. Process for the manufacture of mixed cellulose esters containing glycolyl and acetyl groups, comprising treating materials consisting essentially of cellulose separately with glycollic anhydride and acetic anhydride both in the presence of acylation catalysts and a liquid acylation medium, and subjecting the resulting mixed primary cellulose esters to the action of acidic substances for the purpose of changing their solubility characteristics.

17. Partially hydrolyzed hydroxyalkacetyl esters of cellulose.

18. Partially hydrolyzed cellulose glycollates.

19. Partially hydrolyzed mixed cellulose esters in which part of the nuclear hydroxyl groups are esterified by alkacetyl groups and part by hydroxy-alkacetyl groups.

20. Partially hydrolyzed mixed cellulose esters in which part of the nuclear hydroxyl groups are esterified by acetyl groups and part by glycolyl groups.

HENRY DREYFUS.